

H. Davis.

Pile for Railroad Rails.

No 61,168.

Patented Jan. 15, 1867.

Fig. 2



Fig. 1



Witnesses

F. A. Jackson  
Wm. Treurn

Inventor

Herbert Davis  
Per Mum & Co  
Atty.

# United States Patent Office.

HERBERT DAVIS, OF TROY, NEW YORK.

*Letters Patent No. 61,168, dated January 15, 1867.*

## IMPROVED FAGOT FOR RAILROAD RAIL.

The Schedule referred to in these Letters Patent and making part of the same.

TO ALL WHOM IT MAY CONCERN:

Be it known that I, HERBERT DAVIS, of Troy, in the county of Rensselaer, and State of New York, have invented a new and improved Pile for making Steel-Headed Rail for Railroads; and I do hereby declare that the following is a full, clear, and exact description thereof, which will enable others skilled in the art to make and use the same, reference being had to the accompanying drawings, forming part of this specification, in which—

Figure 1 is an end view of my improved pile.

Figure 2, an end view of a rail rolled from the same.

Similar letters of reference indicate like parts.

This invention relates to a new and useful improvement in the manufacture of steel-headed rails, or those which are composed of an iron neck and base and a steel head or upper surface. The invention consists in a novel manner of forming the pile from which the rail is rolled, whereby the steel head or upper surface is firmly connected to the lower iron portion and effectually prevented from separating under the wear and tear to which the rail is subjected by the action of the car-wheels upon it.

The pile is composed of a series of bars, A A', of iron, of proper dimensions and of rectangular form, laid one upon the other, as shown clearly in fig. 1, and when different qualities of iron are used the bars A' of the better quality are arranged in the pile, as shown clearly in fig. 1, so as to form, when the rail is rolled, an outer coating of superior metal. The upper bars A of the pile are formed with longitudinal grooves, a, and angular projections, b, extending their whole length, and B is a steel cap rolled with a lip or pendent flange, c, at each side, and with angular pendent projections, d, and grooves e at its under side, the flanges c extending down over the sides of the upper bars A, and the projections b of the upper bars fitting in the grooves e of the steel cap, and the projections d of the steel cap fitting in the grooves a of the upper iron bars A. The pile thus formed is properly heated and rolled into a rail by passing it between the usual rollers, and the steel cap B is spread over the entire upper surface of the rail, and extends down at each side of the same nearly to the neck f, as shown clearly in fig. 2. The angular projections and grooves at the under side of the steel cap, and the grooves and projections at the upper sides of the upper bars A, being fitted together as shown, effectually prevent the separation of the steel head from the lower iron portion, as a weld or a union by pressure is not alone depended upon for adhesion. The union of the two different qualities of iron is also an important feature of the invention, as a few bars, A', of superior iron, arranged or disposed with the bars A', of inferior quality, as shown, will form a strong, durable, and economical rail.

Having thus described my invention, I claim as new, and desire to secure by Letters Patent—

The rolling or making of rails for railroads of a pile composed of a series of iron bars, A, provided with a steel cap, B, formed or rolled with a pendent flange at each side, and with longitudinal grooves and projections, e b, at its under surface, and the upper iron bars of the pile rolled or formed with corresponding grooves and projections, a d, to admit of the steel cap and upper iron bars being locked together, substantially as shown and described.

I further claim forming the iron portion of the pile of bars A A' of superior and inferior iron, arranged or disposed substantially in the manner as and for the purpose set forth.

HERBERT DAVIS.

Witnesses:

J. TOWNSEND BURDEN,  
JNO. H. HAYDOCK.